# EUROPEAN PATENT SPECIFICATION

(11) **EP 0 971 371 B1**
(45) Date of publication and mention of the grant of the patent: **12.05.2004**
(21) Application number: 99112688.9
(22) Date of filing: 02.07.1999
(51) Int. Cl.: H01B 9/06

(54) **High voltage direct current electrical cable with mass-impregnated insulation**
Gleichstrom-Hochspannungs-Elektrokabel mit massenimprägnierter Isolierung
Câble électrique courant continu à haute tension avec une isolation impregnée en masse

(30) Priority: 06.07.1998 EP 98112473
(43) Date of publication of application: 12.01.2000
(73) Proprietor: Pirelli & C. S.p.A., 20123 Milano (IT)
(72) Inventor: Bosisio, Claudio, 24100 Brembate Sotto (BG) (IT); Lanfranconi, Gianmario, 24042 Capriate San Gervasio (BG) (IT); Miramonti, Gianni, 20013 Magenta (MI) (IT); Peruzzotti, Franco, 20025 Legnano (MI) (IT)
(74) Representative: Giannesi, Pier Giovanni

(56) References cited:
- US-A- 3 621 110
- US-A- 3 780 206

## Description

The present invention relates to a cable, particularly for carrying high voltage direct current, and suitable for either terrestrial or, in particular, submarine installations, having as insulating layer a material impregnated with an insulating fluid. The present invention further relates to a method for preventing formation of micro-cavities within such an insulating layer.

For the purposes of the present description and the claims, with the term "high voltage" it is meant a voltage of at least 100 kV, preferably of at least 200 kV.

For carrying high voltage direct current, either along terrestrial lines or, in particular, along submarine lines, use is made of cables, commonly known in the art as mass-impregnated cables, in which the conductor, covered with a first semiconducting layer, is electrically insulated by taping with an insulating material, generally paper or multi-layered paper/polypropylene/paper laminates, which is then thoroughly impregnated with a mixture having high electrical resistivity and high viscosity, generally a hydrocarbon oil treated with a viscosity-increasing agent. The cable then comprises a further semiconducting layer and a metal sheath, generally made from lead, which in turn is surrounded by at least one metal armouring structure and one or more protective sheaths made from plastic material.

Although characterized by high reliability in operation even at very high voltages (above 150 kV), mass-impregnated cables have some disadvantages, principally relating to the migration of the insulating fluid within the cable. In particular, during use the cable is subject, owing to variations in the carried current intensity, to thermal cycles which cause migration of the impregnating fluid in radial direction. This is because, when the carried current increases and the cable heats up, the insulating fluid decreases in its viscosity and is subject to a thermal expansion greater than that of all the other components of the cable. This causes a migration of the fluid from the insulating layer towards the exterior, and consequently an increase of the pressure exerted on the metal sheath, which is deformed in the radial direction. When the carried current decreases and the cable cools, the impregnating fluid contracts, while the metal sheath, being constituted by a plastic material (usually lead), remains permanently deformed. Thus there is a decrease of the pressure inside the cable, which causes formation of micro-cavities in the insulating layer, with consequent risk of electrical discharges and therefore of insulation piercing. The risk of piercing increases with an increase of the insulating layer thickness and therefore with an increase of the maximum voltage for which the cable has been designed.

For carrying direct current at high voltage, pressurized cables have been developed, wherein the insulating layer impregnated with the insulating fluid is subjected to a pressure greater than atmospheric pressure, generally above 14 bars, by introducing a pressurized gas, for example nitrogen. Another solution for carrying high voltage direct current consists of fluid oil cables, in which insulation is provided by a pressurized oil with low viscosity and high resistivity (under hydrostatic head). These solutions, although very effective in preventing formation of micro-cavities in the cable insulation, have various disadvantages mainly related to construction complexity, and in particular they cause a limitation of the maximum admissible cable length (generally of not more than 50-100 km). This limitation of the maximum length is a serious drawback, especially in the case of submarine installations, where the required lengths are usually very great.

In Patent GB-2,196,781 a direct current mass-impregnated cable is described, in which a reinforcing structure is present consisting of an elastic tape wound tightly around the metal sheath so as to compensate for radial expansions and contractions of the impregnating oil and consequently to prevent formation of micro-cavities in the insulation. The tape consists of an elastic material of a metal or polymer type, characterized by mechanical hysteresis cycles of the closed type, with a low permanent deformation after thermal cycles.

Patent EP-233,381 describes a high voltage mass-impregnated cable comprising a pressure body consisting of a supporting layer, disposed on the outside of the metal sheath, around which is wound, in at least two overlapping layers, a thin elastic tape made from metal or polymer material. The presence of the supporting layer interposed between the metal sheath and the elastic tape acts as a "bedding", preventing the tape, which is wound with high tension to exert a sufficient containing action on the metal sheath, from damaging the sheath or from eventually causing it to fracture. The risk of fracture increases when the cable overheats, partly owing to the fact that the lead constituting the sheath becomes more malleable, and partly because the cable expands and therefore the tape tension increases.

In the Applicant's perception, both the solutions proposed in the aforesaid patents GB-2,196,781 and EP-233,381 have several drawbacks arising from the fact that the containing tape is disposed on the outside of the metal sheath. Indeed, as explained above, the tension exerted by the tape may damage the sheath and even cause it to fracture, and on the other hand the interposition of a supporting layer between the tape and the sheath, as proposed in patent EP-233,381, not only makes the cable construction more complex, but also decreases effectiveness of the containing action exerted by the said tape on the sheath.

Moreover, the high pressures required to achieve the desired return of the metal sheath during the thermal contraction phase cause a rapid wear of the containing tape, owing to the friction between tape and sheath and between the turns of the tape itself. Finally, the containing tape, being applied externally to the sheath, is subject to the action of external agents, particularly water which may infiltrate under the armour, and this causes a degradation over time of its elastic and mechanical properties.

The Applicant has now found that it is possible to achieve an effective action of containing of the insulating fluid, thus preventing formation of micro-cavities inside the impregnated insulating layer, by winding around the insulating layer beneath the metal sheath at least one tape made from elastomeric semiconducting material, which exerts a compressive action on the insulating layer and acts as a barrier with respect to the radial migration of the insulating fluid without damaging the metal sheath. By contrast with the solutions known in the art, according to the present invention the action of containing of the impregnating fluid is exerted directly on the insulating layer, so that the formation of micro-cavities in the insulation is avoided, even if empty spaces are formed between the cable core and the metal sheath.

The semiconducting properties of the elastomeric material ensure electrical continuity by preventing the creation of potential differences between the core of the cable and the metal sheath, which would lead to electrical discharges and consequently to perforation of the cable. Moreover, the material constituting the tape has a high physical-chemical resistance to the degrading action exerted by the components of the insulating fluid, both in the cold state and, in particular, at the cable operating temperature. This is because the insulating fluid, usually consisting of products of the hydrocarbon type, may cause, especially when hot, a swelling of the elastomeric material and consequently a gradual degradation of elastic and semiconducting properties of the material, with a loss of functionality of the containing layer over time.

In a first aspect, the present invention therefore relates to a cable, particularly for high voltage direct current, comprising an electrical conductor, at least one semiconducting layer, a stratified insulating layer impregnated with an insulating fluid, and a metal sheath disposed on the outside of the said insulating layer, characterized in that between the said insulating layer and the said metal sheath a layer for containing the insulating fluid is provided, comprising at least one winding of a tape made from a semiconducting elastomeric material having a predetermined physical-chemical resistance with respect to the insulating fluid.

In a preferred embodiment, the cable according to the present invention comprises an inner semiconducting layer disposed between the conductor and the insulating layer, and an outer semiconducting layer disposed between the insulating layer and the containing layer.

The physical-chemical resistance of the elastomeric material with respect to the insulating fluid is predetermined so that the elastomeric material, when brought into contact with the insulating fluid, has a low tendency to swell and therefore maintains its elastic and semiconducting properties within values so as to ensure, in normal conditions of use and for a predetermined period of time, preferably throughout the life of the cable, the desired containing action on the insulating layer on the one hand, and the electrical continuity between the cable core and the metal sheath on the other hand.

In a further aspect, the present invention relates to a method for preventing, in a mass-impregnated electrical cable comprising a stratified insulating layer impregnated with an insulating fluid, formation of micro-cavities within the insulating layer, said method comprising winding a tape of an elastomeric material around the said layer so as to form a containing layer for the insulating fluid around the insulating layer.

In a preferred embodiment of the aforesaid method, the tape made from the elastomeric material is disposed between the insulating layer and a metal sheath and has semiconducting properties such that electrical continuity is ensured between the insulating layer and the metal sheath.

To evaluate the physical-chemical resistance of the elastomeric material to the degrading action of the insulating fluid, the Applicant has developed an accelerated ageing test, in which a test specimen of the elastomeric material, put under tension with a predetermined value of percentage elongation, is immersed in the insulating fluid at a predetermined temperature and for a predetermined time. At the end of the ageing period, the test specimen is released, and the permanent percentage elongation, namely the difference in per cent between the length after ageing and the initial length of the test specimen, is determined. The permanent percentage elongation is measured immediately after the release of the test specimen, in other words without allowing the test specimen to recover, at least partially, the initial dimensions over a period of time.

Therefore, the measurement of the permanent percentage elongation constitutes a method for evaluating the residual capacity for elastic recovery after ageing, which must be such as to ensure a sufficient radial compressive force on the impregnated insulating layer in the presence of thermal cycles of expansion and contraction which the cable undergoes during use.

On the basis of the experiments carried out by the Applicant, it is believed, in particular, the elastomeric material has the desired resistance to degradation of the elastic properties due to contact with the insulating fluid if a test specimen of the material, kept under tension with an imposed elongation of 50% and immersed in the insulating fluid for 360 days at 85°C, has a permanent elongation of less than 35%, preferably less than 25%.

This quantitative indication is provided purely for illustrative purposes, and it is possible for a person skilled in the art to find different criteria which can be used to evaluate the physical-chemical resistance of the elastomeric material with respect to the insulating fluid as a function of the specific design of the cable to be made, the materials used and the operating conditions of the cable.

The elastomeric base material to be used for making the containing layer according to the present invention may be selected, for example, from: nitrile rubbers, styrene rubbers, fluoroelastomers, silicone rubbers, ethylene/propylene (EPR) or ethylene/propylene/diene (EPDM) elastomers, elastomeric copolymers of ethylene with ethylenically unsaturated esters, polychloro-sulphonated or polychlorinated elastomers, and the like, or mixtures thereof. The following are particularly preferred:
- butadiene/acrylonitrile copolymers, particularly butadiene/acrylonitrile copolymers with a high content of acrylonitrile (generally from 20% to 45% by weight of acrylonitrile), preferably in an at least partially hydrogenated form;
- ethylene/vinylacetate, ethylene/methylacrylate, ethylene/ethylacrylate or ethylene/butylacrylate copolymers with a high ester content (generally from 28% to 80% by weight);
- fluoroelastomers based on tetrafluoroethylene and/or vinylidene fluoride with hexafluoropropene and/or perfluorovinyl ethers;
- polychloroethylene, polychlorosulphonylethylene, polychloroprene, and the like.

The elastomeric material may be vulcanized by known methods, for example by sulphur cross-linking, or via radicals. Preferably, elastomeric materials having a high cross-linking degree are used, so as to achieve high elastic performance. Preferably, the elastomeric material as such (i.e. before ageing in contact with the insulating fluid) has stress at break greater than 15 MPa, preferably greater than 20 MPa, elongation at break greater than 300%, preferably greater than 400%, and modulus at 100% greater than 3 MPa, preferably greater than 3.5 MPa.

To impart semiconducting properties to the elastomeric material, it is possible to use products known in the art for the preparation of semiconducting polymer compositions. In particular, an electrically conducting carbon black may be used having a surface area generally greater than 20 m²/g, for example electroconducting acetylene or furnace black, and the like, or also high-conductivity carbon black, having for example a surface area of at least 900 m²/g.

The amount of carbon black to be added to the mixture is such as to impart sufficient semiconducting properties to the final elastomeric material, and in particular to provide a volume resistivity of the elastomeric material, measured at ambient temperature, of less than 100 Ω·m, preferably less than 5 Ω·m. Typically, the quantity of carbon black may vary from 5 to 70%, preferably from 10 to 50%, by weight with respect to the weight of the polymer.

Other additives of various kinds known in the art, such as plasticizers, antioxidants, cross-linking accelerators, co-vulcanizing agents, etc., are usually added to the polymer mixture.

The attached figures show an embodiment of the cable according to the present invention, wherein:
Fig. 1 shows a perspective view of a section of a cable according to the present invention with portions partially removed to show its structure;
Fig. 2 shows a transverse section through the cable shown in Fig. 1;
Figs. 3 and 4 show a schematic sectional representation of two possible embodiments of the taping with the elastomeric material.

With reference to the aforesaid figures, the cable (1) according to the present invention comprises, in sequence from the centre to the exterior, a conductor (2), an inner semiconducting layer (3), a stratified insulating layer (4), an outer semiconducting layer (5), a containing layer (6) comprising one or more tapes (7) of elastomeric material wound around the inner semiconducting layer (5), and a metal sheath (8).

The conductor (2) generally consists of a plurality of single conductors, preferably made from copper or aluminium, for example in the form of wires stranded together by conventional methods, or, preferably, is of the copper-wedge or Milliken type (as shown in Fig. 1), in which a plurality of metal conductors (21) are joined together so as to form individually insulated sectors in order to minimize stray currents. A duct (22) allowing the insulating fluid to move longitudinally along the cable may be present in the centre of the conductor (2).

Around the conductor (2) there is a layer (3) having semiconducting properties, consisting, for example, of windings of cellulose paper tapes filled with semiconducting carbon black.

The insulating layer (4) generally consists of windings of cellulose paper tapes, having a density typically in the range of from 0.7 to 1.2 g/cm³, preferably from 0.9 to 1.1 g/cm³. Instead of the cellulose paper, paper/polypropylene/paper laminates may be used as described, for example, in patents GB-1,045,527 and US-4,602,121, or in patent application EP-684,614.

The windings of the insulating layer (4) are impregnated with an insulating fluid generally having a viscosity of from 50 to 300 cSt at 100°C, and of from 500 to 10,000 cSt at 60°C, and an electrical resistivity generally greater than 1·10¹⁴ Ω·m. Fluids of this type generally consist of a mineral oil of naphthenic or paraffin type, or mixtures thereof, to which a viscosity-increasing agent is added in amounts usually of from 0.5% to 10% by weight, preferably from 1% to 5% by weight. The viscosity-increasing additives may be selected, for example, from: high molecular weight polyolefins, for example polyisobutenes; polymerized colophonic resins; micro-crystalline wax; elastomeric materials in a subdivided form, for example styrene or isoprene rubbers; and similar.

The insulating layer (4) generally consists of windings of cellulose paper tapes, having a density typically in the range of from 0.7 to 1.2 g/cm³, preferably from 0.9 to 1.1 g/cm³. Instead of the cellulose paper, paper/polypropylene/paper laminates may be used as described, for example, in patents GB-1,045,527 and US-4,602,121, or in patent application EP-684,614.

The windings of the insulating layer (4) are impregnated with an insulating fluid generally having a viscosity of from 50x10⁻⁶ to 300x10⁻⁶ m²/s (cSt) at 100°C, and of from 500x10⁻⁶ m²/s to 10,000x10⁻⁶ m²/s (cSt) at 60°C, and an electrical resistivity generally greater than 1·10¹⁴ Ω·m. Fluids of this type generally consist of a mineral oil of naphthenic or paraffin type, or mixtures thereof, to which a viscosity-increasing agent is added in amounts usually of from 0.5% to 10% by weight, preferably from 1% to 5% by weight. The viscosity-increasing additives may be selected, for example, from: high molecular weight polyolefins, for example polyisobutenes; polymerized colophonic resins; micro-crystalline wax; elastomeric materials in a subdivided form, for example styrene or isoprene rubbers; and similar.

The containing layer (6) is formed around the outer semiconducting layer (5) by spirally winding the tape (7) made from the elastomeric material as described above. The surface of the tape is as smooth and defect-free as possible, so that optimal contact between overlapping turns of the tape is achieved, and therefore infiltration of insulating fluid is prevented.

The winding preferably consists of one or more layers of the tape wound with an overlap between successive turns of at least 20%, preferably at least 50%, with respect to the tape width, so that the possibility of infiltration of the impregnating fluid between one turn and the next is prevented. An overlap of this type ensures a certain safety During the process of winding around the cable core, a traction force is applied to the tape so as to exert on the underlying layers a radial pressure sufficient to obtain an effective action of containment of the impregnating fluid. In general, the tape is wound with a traction force such that an elongation of the tape generally of from 40% to 90%, preferably of from 50% to 70%, is obtained.

The metal sheath (8), usually made from lead or lead alloys, encloses the cable core consisting of the aforementioned elements, and any space within the sheath (8) is filled by the insulating fluid so as to thoroughly impregnate the cable layers, and in particular the stratified insulating layer (4).

Around the sheath (8) an armoured structure (not shown in the figures) is disposed, capable of protecting the cable from the high hydrostatic pressures to which it is subjected during use in submarine applications. This armoured structure may comprise, for example, a sheath made from plastic material to which a metal sheath, made e.g. from steel wires, is applied, which in turn is protected by an external sheath, also made from a plastic material. The armoured structure may also comprise one or more layers of padding to prevent the metal armour from damaging the adjacent layers.

An example of a polymer mixture suitable for making the containing layer according to the present invention is as follows:
- nitrile rubber (NBR): 50.0% by weight butadiene/acrylonitrile copolymer (33% acrylonitrile by weight), having Mooney viscosity ML (1+4) at 100°C = 45 ±5
   (product Krynac® 34-50 by Bayer);
- liquid nitrile rubber (plasticizer), 10.7% by weight having a Brookfield viscosity of 20,000-30,000 cP (at 12 rpm, 50°C, needle no. 4)
- conducting carbon black: 32.0% by weight product Vulcan® XC 72 by Cabot;
- sulphur (cross-linking agent): 0.6% by weight product Rhenogran® S-80 (80% sulphur pre-dispersion) by Rhein Chemie;
- zinc oxide (co-vulcanizing agent): 5.0% by weight product Zinc Oxide S.O. by A-Esse;
- tetramethylthiuram disulphide (TMTD) 1.5% by weight (vulcanization accelerator) :
   product Rhenogran® TMTD-80 (pre-dispersion with 80% TMTD) by Rhein Chemie;
- 2,2,4-trimethyl-1,2-dihydroquinoline 0.2% by weight (TMQ) (antioxidant):
   product Anox® HB by Great Lakes.

The mixture was prepared by means of a Banbury mixer, then calendered and cross-linked by heating at 160°C for 30 minutes. From the so produced sheet, dumb-bell test specimens with dimensions 90 x 15 x 1.5 mm were prepared. On a test specimen in the initial state, volume resistivity (by means of a Metra Hit 16 multimeter by ABB) and mechanical properties (by means of instrument Instron 1122, with a traction rate of 25 mm/min.) were determined. The test specimens were subjected to traction with an elongation of 50% and kept immersed in an insulating fluid for predetermined increasing periods at a temperature of 85°C. The fluid is of the type commonly used for mass-impregnated cables (commercial product T2015 by Dussek-Campbell), based on mineral oil with the addition of approximately 2% by weight of a high molecular weight polyisobutene as viscosity-increasing agent.

At the end of each period of immersion, one test specimen was removed from the insulating fluid, left to cool to ambient temperature (still under traction), and cleaned with petroleum ether so as to eliminate fluid residues, and its volume resistivity was measured as indicated above. After removing the traction force, permanent elongation was immediately measured and the mechanical properties were then determined as indicated above. Another set of test specimens was subjected to the same measurements in the conditions indicated above, but with an imposed elongation of 75%.

The results of the two sets of tests are shown in Tables 1 and 2. These results clearly demonstrate that the elastomeric material used maintains its elastic properties within satisfactory values even after prolonged immersion in the insulating fluid at high temperature in stretching conditions.

**TABLE 1**

| Period of immersion in T2015 (days) | Imposed elongation: 50% | | | | |
|---|---|---|---|---|---|
| | Resistivity (Ω m) | Permanent elongation (%) | Stress at break (MPa) | Elongation at break (%) | Modulus at 100% (MPa) |
| 0 | 0.85 | -- | 21.0 | 435 | 4.0 |
| 30 | 0.66 | 14.4 | 16.4 | 330 | 4.83 |
| 60 | 1.03 | 11.1 | 16.2 | 310 | 4.4 |
| 120 | 0.88 | 18.8 | 16.1 | 280 | 4.5 |
| 150 | 2.07 | 19.0 | 14.7 | 230 | 4.51 |
| 240 | 3.10 | 24.0 | 14.0 | 220 | 4.7 |
| 360 | 2.91 | 23.0 | 14.1 | 230 | 4.75 |

**TABLE 2**

| Period of immersion in T2015 (days) | Imposed elongation: 75% | | | | |
|---|---|---|---|---|---|
| | Resistivity (Ω m) | Permanent elongation (%) | Stress at break (MPa) | Elongation at break (%) | Modulus at 100% (MPa) |
| 0 | 0.85 | -- | 21.0 | 435 | 4.0 |
| 30 | 0.70 | 24.4 | 21.4 | 335 | 4.4 |
| 60 | 1.20 | 18.8 | 19.5 | 360 | 4.3 |
| 120 | 1.75 | 33.3 | 15.1 | 250 | 4.5 |
| 150 | 3.29 | 43.0 | 16.1 | 220 | 4.6 |
| 240 | 2.80 | 45.5 | 14.7 | 220 | 4.6 |
| 360 | 2.70 | 44.6 | 14.8 | 230 | 4.7 |

## Claims

1. Cable (1), particularly for carrying high voltage direct current, comprising an electrical conductor (2), at least one semiconducting layer (3,5), a stratified insulating layer (4) impregnated with an insulating fluid, and a metal sheath (8) disposed on the outside of the said insulating layer (4), **characterized in that** between the said insulating layer (4) and the said metal sheath (8) a layer (6) for containing the insulating fluid is provided, comprising at least one winding of a tape (7) made from a semiconducting elastomeric material having a predetermined physical-chemical resistance with respect to the insulating fluid.

2. Cable according to Claim 1, comprising an inner semiconducting layer (3) disposed between the conductor (2) and the insulating layer (4), and an outer semiconducting layer (5) disposed between the insulating layer (4) and the containing layer (6).

3. Cable according to any of the preceding claims, wherein the elastomeric material has a physical-chemical resistance of the elastomeric material with respect to the insulating fluid such that a test specimen of the elastomeric material, when placed under traction with a predetermined percentage elongation and immersed in the insulating fluid at a predetermined temperature for a predetermined time, shows a permanent percentage elongation below a predetermined value.

4. Cable according to Claim 3, wherein the test specimen of elastomeric material, kept under traction with an imposed elongation of 50% and immersed in the insulating fluid for 360 days at 85°C, has a permanent elongation of less than 35%.

5. Cable according to Claim 4, wherein the test specimen of elastomeric material, kept under traction with an imposed elongation of 50% and immersed in the insulating fluid for 360 days at 85°C, has a permanent elongation of less than 25%.

6. Cable according to anyone of the preceding claims, wherein the elastomeric material is selected from: nitrile rubbers, styrene rubbers, fluoroelastomers, silicone rubbers, ethylene/propylene (EPR) or ethylene/propylene/diene (EPDM) elastomers, elastomeric copolymers of ethylene with ethylenically unsaturated esters, polychlorosulphonated or polychlorinated elastomers, and the like, or mixtures thereof.

7. Cable according to Claim 6, wherein the elastomeric material is a butadiene/acrylonitrile copolymer with from 20% to 45% by weight of acrylonitrile.

8. Cable according to Claim 7, wherein the butadiene/acrylonitrile copolymer is at least partially hydrogenated.

9. Cable according to Claim 6, wherein the elastomeric material is an ethylene/vinylacetate, ethylene/methylacrylate, ethylene/ethylacrylate or ethylene/butylacrylate copolymer having a ester content of from 28% to 80% by weight.

10. Cable according to Claim 6, wherein the elastomeric material is a fluoroelastomer based on tetrafluoroethylene and/or vinylidene fluoride with hexafluoropropene and/or perfluorovinyl ethers.

11. Cable according to Claim 6, wherein the elastomeric material is selected from: polychloroethylene, polychlorosulphonyl ethylene, and polychloroprene.

12. Cable according to anyone of Claims 6 to 11, wherein the elastomeric material is vulcanized by sulphur cross-linking.

13. Cable according to anyone of Claims 6 to 11, wherein the elastomeric material is vulcanized via radicals.

14. Cable according to anyone of the preceding claims, wherein the elastomeric material has a stress at break greater than 15 MPa, an elongation at break greater than 300%, and a modulus at 100% greater than 3 MPa.

15. Cable according to anyone of the preceding claims, wherein the containing layer (6) consists of one or more layers of the tape (7) of the elastomeric material wound with an overlap between successive turns of at least 20% with respect to the tape width.

16. Cable according to Claim 15, wherein the containing layer (6) consists of one or more layers of the tape (7) of the elastomeric material wound with an overlap between successive turns of at least 50% with respect to the tape width.

17. Cable according to anyone of Claims 1 to 14, wherein the containing layer (6) comprises at least two tape layers (7) wound spirally with turns abutting each other without substantial overlap.

18. Cable according to anyone of the preceding claims, wherein the tape (7) of the elastomeric material is wound with a traction force such that an elongation of the tape of from 40% to 90% is obtained.

19. Cable according to Claim 18, wherein the tape (7) of the elastomeric material is wound with a traction force such that an elongation of the tape of from 50% to 70% is obtained.

20. Method for preventing, in cable (1) comprising an electrical conductor (2), at least one semiconducting layer (3,5), a stratified insulating layer (4) impregnated with an insulating fluid, and a metal sheath (8) disposed on the outside of the said insulating layer (4), formation of micro-cavities within the insulating layer (4), said method comprising winding a tape (7) of an elastomeric material around the said layer so as to form a containing layer (6) for the insulating fluid around the insulating layer (4).

21. Method according to Claim 20, wherein the tape (7) made from the elastomeric material is disposed between the insulating layer (4) and a metal sheath (8) and has semiconducting properties such that electrical continuity is ensured between the insulating layer (4) and the metal sheath (8).

## Patentansprüche

1. Kabel (1), insbesondere zum Führen eines Hochspannungs-Gleichstroms, das einen elektrischen Leiter (2), mindestens eine halbleitende Schicht (3, 5), eine Lagenisolierungsschicht (4), die mit einer Isolierungsflüssigkeit imprägniert ist, und einen Metallmantel (8), der an der Aussenseite der Isolierungsschicht (4) angeordnet ist, umfasst, **dadurch gekennzeichnet, dass** zwischen der Isolierungsschicht (4) und dem Metallmantel (8) eine Schicht (6) zur Eingrenzung der Isolierungsflüssigkeit vorgesehen ist, die mindestens eine Wicklung eines Bandes (7) umfasst, das aus einem halbleitenden elastomeren Material mit einer vorgegebenen physikalisch-chemischen Beständigkeit gegenüber der Isolierungsflüssigkeit hergestellt ist.

2. Kabel gemäss Anspruch 1, das eine innere halbleitende Schicht (3), die zwischen dem Leiter (2) und der Isolierungsschicht (4) angeordnet ist, und eine äussere halbleitende Schicht (5), die zwischen der Isolierungsschicht (4) und der Eingrenzungsschicht (6) angeordnet ist, umfasst.

3. Kabel gemäss mindestens einem der vorstehenden Ansprüche, wobei das elastomere Material eine solche physikalisch-chemische Beständigkeit des elastomeren Materials gegenüber der Isolierungsflüssigkeit besitzt, dass ein Teststück des elastomeren Materials, wenn es mit einer vorgegebenen prozentualen Dehnung unter Zug gesetzt wird und bei einer vorgegebenen Temperatur für eine vorgegebene Zeit in die Isolierungsflüssigkeit eingetaucht wird, eine bleibende prozentuale Dehnung unter einem vorgegebenen Wert zeigt.

4. Kabel gemäss Anspruch 3, wobei das Teststück des elastomeren Materials, das unter Zug mit einer erzwungenen Dehnung von 50 % gehalten wird und für 360 Tage bei 85°C in die Isolierungsflüssigkeit eingetaucht wird, eine bleibende Dehnung von weniger als 35 % aufweist.

5. Kabel gemäss Anspruch 4, wobei das Teststück des elastomeren Materials, das unter Zug mit einer erzwungenen Dehnung von 50 % gehalten wird und für 360 Tage bei 85°C in die Isolierungsflüssigkeit eingetaucht wird, eine bleibende Dehnung von weniger als 25 % aufweist.

6. Kabel gemäss mindestens einem der vorstehenden Ansprüche, wobei das elastomere Material ausgewählt ist aus: Nitrilkautschuk, Styrolkautschuk, Fluorelastomeren, Siliconkautschuk, Ethylen/Propylen(EPR) oder Ethylen/Propylen/Dien (EPDM)-Elastomeren, elastomeren Copolymeren von Ethylen mit ethylenisch ungesättigten Estern, polychlorsulfonierten oder polychlorierten Elastomeren und dergleichen oder Mischungen davon.

7. Kabel gemäss Anspruch 6, wobei das elastomere Material ein Butadien/Acrylnitril-Copolymer mit 20 bis 45 Gew.% Acrylnitril ist.

8. Kabel gemäss Anspruch 7, wobei das Butadien/Acrylnitril-Copolymer zumindest teilweise hydriert ist.

9. Kabel gemäss Anspruch 6, wobei das elastomere Material ein Ethylen/Vinylacetat-, Ethylen/Methylacrylat-, Ethylen/Ethylacrylat- oder Ethylen/Butylacrylat-Copolymer mit einem Estergehalt von 28 bis 80 Gew.% ist.

10. Kabel gemäss Anspruch 6, wobei das elastomere Material ein Fluorelastomer auf Basis von Tetrafluorethylen und/oder Vinylidenfluorid mit Hexafluorpropen und/oder Perfluorvinylethern ist.

11. Kabel gemäss Anspruch 6, wobei das elastomere Material ausgewählt ist aus Polychlorethylen, Polychlorsulfonylethylen und Polychloropren.

12. Kabel gemäss mindestens einem der Ansprüche 6 bis 11, wobei das elastomere Material durch Vernetzung mit Schwefel vulkanisiert ist.

13. Kabel gemäss mindestens einem der Ansprüche 6 bis 11, wobei das elastomere Material mittels Radikalen vulkanisiert ist.

14. Kabel gemäss mindestens einem der vorstehenden Ansprüche, wobei das elastomere Material eine Bruchspannung von grösser als 15 MPa, eine Bruchdehnung von grösser als 300 % und einen Modul bei 100 % von grösser als 3 MPa besitzt.

15. Kabel gemäss mindestens einem der vorstehenden Ansprüche, wobei die Eingrenzungsschicht (6) aus einer oder mehreren Schichten des Bandes (7) des elastomeren Materials besteht, das mit einer Überlappung zwischen aufeinanderfolgenden Windungen von mindestens 20 % in bezug auf die Bandbreite aufgewickelt ist.

16. Kabel gemäss Anspruch 15, wobei die Eingrenzungsschicht (6) aus einer oder mehreren Schichten des Bandes (7) des elastomeren Materials besteht, das mit einer Überlappung zwischen aufeinanderfolgenden Windungen von mindestens 50 % in bezug auf die Bandbreite aufgewickelt ist.

17. Verfahren gemäss mindestens einem der Ansprüche 1 bis 14, wobei die Eingrenzungsschicht (6) mindestens zwei Bandschichten (7) umfasst, die spiralförmig gewunden sind, wobei die Windungen ohne wesentliche Überlappung aneinandergrenzen.

18. Kabel gemäss mindestens einem der vorstehenden Ansprüche, wobei das Band (7) des elastomeren Materials mit einer solchen Zugkraft aufgewickelt ist, dass eine Dehnung des Bandes von 40 bis 90 % erhalten wird.

19. Kabel gemäss Anspruch 18, wobei das Band (7) des elastomeren Materials mit einer solchen Zugkraft aufgewickelt ist, dass eine Dehnung des Bandes von 50 bis 70 % erhalten wird.

20. Verfahren zur Vermeidung der Bildung von Mikrohohlräumen innerhalb der Isolierungsschicht (4) in einem Kabel (1), das einen elektrischen Leiter (2), mindestens eine halbleitende Schicht (3, 5), eine Lagenisolierungsschicht (4), die mit einer Isolierungsflüssigkeit imprägniert ist, und einen an der Aussenseite der Isolierungsschicht (4) angeordneten Metallmantel (8) umfasst, wobei das Verfahren das Aufwickeln eines Bandes (7) eines elastomeren Materials um die Schicht herum umfasst, um so eine Eingrenzungsschicht (6) für die Isolierungsflüssigkeit um die Isolierungsschicht (4) herum auszubilden.

21. Verfahren gemäss Anspruch 20, wobei das Band (7), das aus dem elastomeren Material gefertigt ist, zwischen der Isolierungsschicht (4) und einem Metallmantel (8) angeordnet ist und Halbleitereigenschaften aufweist, so dass der elektrische Durchgang zwischen der Isolierungsschicht (4) und dem Metallmantel (8) sichergestellt ist.

## Revendications

1. Câble (1), destiné en particulier à véhiculer du courant continu sous haute tension, comprenant un conducteur électrique (2), au moins une couche semi-conductrice (3,5), une couche isolante stratifiée (4) imprégnée de fluide isolant, et une gaine métallique (8) placée sur le coté extérieur de ladite couche isolante (4), **caractérisé en ce que** entre ladite couche isolante (4) et ladite gaine métallique (8), il y a couche (6) destiner à confiner le fluide isolant et comprenant au moins un enroulement de ruban (7) préparé à partir d'un matériau élastomère semiconducteur présentant une résistance physico-chimique prédéterminée vis-à-vis du fluide isolant.

2. Câble selon la revendication 1, comprenant une couche interne semi-conductrice (3) placée entre le conducteur (2) et la couche isolante (4), et une couche externe semi-conductrice (5) placée entre la couche isolante (4) et la couche de confinement (6).

3. Câble selon l'une quelconque des revendications précédentes, dans lequel le matériau élastomère présente vis-à-vis du fluide isolant une résistance physico-chimique telle que lorsqu'un échantillon du matériau élastomère est soumis à une traction provoquant un pourcentage d'allongement prédéterminé et immergé dans le fluide isolant à une température prédéterminée pendant un temps prédéterminé, il présente un pourcentage d'allongement permanent inférieur à une valeur prédéterminée.

4. Câble selon la revendication 3, dans lequel l'échantillon de matériau élastomère, soumis à une traction provoquant un allongement fixé à 50 % et immergé dans le fluide isolant pendant 360 jours à 85 °C, présente un pourcentage d'allongement permanent inférieur à 35 %.

5. Câble selon la revendication 4, dans lequel l'échantillon de matériau élastomère, soumis à une traction provoquant un allongement fixé à 50 % et immergé dans le fluide isolant pendant 360 jours à 85 °C, présente un pourcentage d'allongement permanent inférieur à 25 %.

6. Câble selon l'une quelconque des revendications précédentes, dans lequel le matériau élastomère est choisi dans l'ensemble constitué par : les caoutchoucs nitrile, les caoutchoucs de styrène, les élastomères fluorés, les caoutchoucs de silicone, les élastomères éthylène/propylène (EPR) ou éthylène/propylène/diène (EPDM), les élastomères copolymères d'éthylène et d'esters à insaturation éthyléniques, les élastomères polychlorosulfonés ou polychlorés, et autres similaires, et leurs mélanges.

7. Câble selon la revendication 6, dans lequel le matériau élastomère est un copolymère butadiène/acrylonitrile comportant 20 % à 45 % en poids d'acrylonitrile.

8. Câble selon la revendication 7, dans lequel le copolymère de butadiène/acrylonitrile est au moins partiellement hydrogéné.

9. Câble selon la revendication 6, dans lequel le matériau élastomère est un copolymère éthylène(acétate de vinyle), éthylène(acrylate de méthyle), éthylène(acrylate d'éthyle) ou éthylène(acrylate de buthyle) comportant de 28 % à 80 % en poids d'ester.

10. Câble selon la revendication 6, dans lequel le matériau élastomère est un élastomère fluoré à base de tétrafluoroéthylène, et/ou de fluorure de vinylidène, accompagné d'hexafluoropropène et/ou d'éthers de perfluorovinyle.

11. Câble selon la revendication 6, dans lequel le matériau élastomère est choisi dans l'ensemble constitué par les polychloroéthylène, polychlorosulfonyléthylène et polychloropropène.

12. Câble selon l'une quelconque des revendications 6 à 11, dans lequel le matériau élastomère est vulcanisé par réticulation au soufre.

13. Câble selon l'une quelconque des revendications 6 à 11, dans lequel le matériau élastomère est vulcanisé par voie radicalaire.

14. Câble selon l'une quelconque des revendications précédentes, dans lequel le matériau élastomère présente une tension à la rupture supérieure à 15 MPa, un allongement à la rupture supérieur à 300 %, et un module à 100 % supérieur à 3 MPa.

15. Câble selon l'une quelconque des revendications précédentes, dans lequel la couche de confinement (6) consiste en une ou plusieurs couches de ruban (7) de matériau élastomère enroulées avec un taux de recouvrement entre deux spires successifs d'au moins 20 % par rapport à la largeur du ruban.

16. Câble selon la revendication 15, dans lequel la couche de confinement (6) consiste en une ou plusieurs couches de ruban (7) de matériau élastomère enroulées avec un taux de recouvrement entre deux spires successifs d'au moins 50 % par rapport à la largeur du ruban.

17. Câble selon l'une quelconque des revendications 1 à 14, dans lequel la couche de confinement (6) comprend au moins deux couches de ruban (7) enroulées en spirale avec des spires en contact les unes avec les autres sans recouvrement sensible.

18. Câble selon l'une quelconque des revendications précédentes, dans lequel le ruban (7) de matériau élastomère est enroulé avec une force de traction telle que le ruban allongé 40 % à 90 %.

19. Câble selon la revendication 18, dans lequel le ruban (7) de matériau élastomère est enroulé avec une force de traction telle que le ruban s'allonge de 50 % à 70 %.

20. Procédé permettant, dans un câble (1) comprenant un conducteur électrique (2), au moins une couche semi-conductrice (3,5), une couche isolante stratifiée (4) imprégnée de fluide isolant, et une gaine métallique (8) placée sur le coté extérieur de ladite couche isolante (4), d'éviter la formation de micro-cavités dans la couche isolante (4), ledit procédé comprenant le fait d'enrouler d'un ruban (7) de matériau élastomère autour de ladite couche de façon à former une couche (6) confinant le fluide isolant autour de la couche isolante (4).

21. Procédé selon la revendication 20, dans lequel le ruban (7) préparé à partir de matériau élastomère est placé entre la couche isolante (4) et la gaine métallique (8) et présente des propriétés semiconductrices qui assurent la continuité électrique entre la couche isolante (4) et la gaine métallique (8).
